

No. 836,464.

PATENTED NOV. 20, 1906.

P. SCHMID.

PROCESS OF UNGUMMING AND DYEING RAW NATURAL SILK.

APPLICATION FILED JAN. 27, 1906.



Witnesses.

J. H. Kline  
William J. Firth

Inventor:  
Peter Schmid

Henry Compton  
Attorney

# UNITED STATES PATENT OFFICE.

PETER SCHMID, OF BASEL, SWITZERLAND.

## PROCESS OF UNGUMMING AND DYEING RAW NATURAL SILK.

No. 836,464.

Specification of Letters Patent.

Patented Nov. 20, 1906.

Application filed January 27, 1906. Serial No. 299,153.

*To all whom it may concern:*

Be it known that I, PETER SCHMID, a citizen of the Swiss Republic, and a resident of Basel, Switzerland, have invented a new and useful Process for Ungumming and Dyeing Raw Natural Silk, of which the following is a full, clear, and exact specification.

I have found that natural silk, natural-silk waste, and yarns and tissues of natural silk or of natural-silk waste can be ungummed and dyed simultaneously by the same operation when the said raw silk is treated during a convenient time with the lather of a soapy dyeing-bath in the presence of air and steam and afterward submitted to a single washing.

For ungumming and dyeing, for example, one hundred kilograms of raw-silk hanks I proceed as follows: In the upper part of a not 20 tightly-closed vessel—for instance, the vessel *a* of the apparatus shown in the annexed drawing—containing about five hundred and eighty liters of water in which about thirty-three kilograms of soap and about five 25 kilograms of a rhodamine dyestuff have been dissolved the silk hanks are suspended or laid in convenient holders—as, for instance, the sieves *b* of the annexed drawing—in such manner that the liquid *c* of the vessel may 30 not at any rate come into contact with the silk hanks. The soapy dyeing-bath of the vessel is then heated by steam or otherwise—for instance, by the serpentine pipe *d* of the annexed drawing—to the boiling-point in 35 order to transform it in lather which will rise in the vessel along the hanks contained therein and envelop the latter at all parts, so that the said hanks will be subjected to the combined action of steam, hot air, and lather 40 of the soapy dyeing-bath, the effect of which will be to soften and render permeable the gumming envelop (sericine envelop) of the silk, so that the dyestuff of the lather may penetrate to the inner fibroin of the silk and 45 be fixed by the said fibroin after twenty to fifty minutes. The hanks are then removed with their holders from the vessel and washed in water, whereby the softened sericine is completely or only partly removed 50 from the fibroin.

The transformation of the soapy dyeing-bath in lather may be aided by injecting air

under pressure—for instance, by the perforated serpentine pipe *e*, supplied with pressure-air—in the said bath contained in 55 the under part of the vessel.

A part of the sericine may without inconvenience remain on the fibroin.

To the soapy dyeing-bath charging substances—as, for instance, substances containing tannin, as catechu, divi-divi, sumac, &c., metallic salts, as tin salts, lead salts, antimony salts, &c.—may be added in order to charge also the silk with these substances during the ungumming and dyeing process. 55

What I claim is—

1. The herein-described process for ungumming and dyeing silk simultaneously, consisting in first making a bath containing soap and a dye, then treating the raw silk 70 with lather of the said bath in presence of steam and air, and finally washing the silk thus treated.

2. The herein-described process for ungumming and dyeing silk simultaneously, 75 consisting in first making a bath containing soap and a dye, then treating the raw silk with lather of the said bath obtained by heating the said soapy dyeing-bath to the boiling-point in presence of air, and in finally 80 washing the silk thus treated.

3. The herein-described process for ungumming and dyeing silk simultaneously, 85 consisting in first making a bath containing soap and a dye, then treating the raw silk with lather of the said bath, obtained by heating the said soapy dyeing-bath to the boiling-point and by injecting air in the said soapy dyeing-bath, and finally washing the silk thus treated. 90

4. The described process for ungumming and dyeing silk simultaneously, consisting in first making a bath containing soap, a dye and charging substances, then treating the raw silk with lather of the said bath in presence of steam and air, and finally washing the silk thus treated. 95

In witness whereof I have hereunto signed my name, this 18th day of January, 1906, in the presence of two subscribing witnesses. 100

PETER SCHMID.

Witnesses

GEO. GIFFORD,  
AMAND RITTER.